

1

3,317,273

**METALLIZING AZOIC DYEINGS AND PRINTS**  
 Clemens Streck, Loudonville, N.Y., assignor to General  
 Aniline & Film Corporation, New York, N.Y., a corpora-  
 tion of Delaware  
 No Drawing. Filed Apr. 16, 1964, Ser. No. 360,436  
 14 Claims. (Cl. 8—42)

This application is a continuation-in-part of application Ser. No. 175,799, of Clemens Streck, filed Feb. 26, 1962.

The present invention relates to, in general, the metallization of azoic dyeings and prints and, in particular, to an improved method for the metallization of azoic dyeings on the fiber.

Previous arrangements and methods heretofore considered practical contemplated pre-metallization of water-soluble dyes in an alkali metal ion-containing dye bath solution and subsequently dyed on or into the fiber. The conditions under which dyeing of fibers with pre-metallized dyes are usually very stringent involving boiling of the fabric to be dyed for several hours. Metallization treatments of previously dyed fibrous materials, on the other hand, is preferable since dyeings are obtained having improved light fastness and improved shades. Also such treatments lend themselves to continuous operations. However, such metallization treatments are delicate and certain precautions must be exercised since the treatment must be sufficiently drastic to effect metallization but insufficient to tender or damage the fiber. Additionally, in order for such treatments to be adapted to continuous operations a sufficiently loose metal complex must be employed. Yet the metal complex must be sufficiently stable under the conditions of application so as not to precipitate out of solution.

Accordingly, it is an object of this invention to provide an improved method for the metallization of azoic dyeings and prints.

A further object of this invention resides in the provision of an improved method for the metallization of azoic dyeings and prints which can be carried out in a continuous fashion.

Yet another object of this invention is to provide azoic printings and dyeings of improved light fastness which are substantially free of light breaks and fading.

Still another object of this invention contemplates the provision of improved metallizing compositions suitable for metallizing azoic dyeings and printed fibers.

Other objects and advantages of the invention will become further apparent hereinafter as the description of the invention proceeds.

It has now been discovered that the aforesaid objects can be readily accomplished by treating a fibrous material dyed with a water-insoluble azoic dye free of solubilizing groups and containing in o,o'-positions relative to an azo linkage groups capable of conversion to a complex metal compound with an alkali-ion-free aqueous alkaline solution, having a pH in the range of above 7—9, containing a metallizing compound of the group consisting of salts and hydroxides of copper, cobalt, and nickel capable of forming a metal complex with said azoic dye and ammonium salt of the formula:



wherein X represents a member selected from the group consisting of hydroxyl, hydrogen and alkyls having 1 to 4 carbon atoms and such amount of ammonium hydroxide as is necessary to maintain the pH of the solution in said range.

The metallizing compounds capable of forming a metal complex with said azoic dyeing or printing which can be

2

advantageously employed are the water-soluble or disperible salts and hydroxides of copper, nickel or cobalt, usually in the form of the chlorides, sulfates, nitrates, formates, acetates, propionates and butyrates.

5 The amount of metallizing compound which may be employed will usually depend upon the degree of metallization desired. While molar ratios are required for complete metallization, the amount employed can be varied from an equivalent to an excess of one equivalent of metal per equivalent of dye.

The metallizing compound is coordinated by the addition to an aqueous solution thereof of an ammonium salt characterized by the formula above. This ammonium salt can be added as such or if desired, can be added as 15 the corresponding free acid and ammonium hydroxide be then added to form the ammonium salt by neutralization; in any event sufficient ammonium hydroxide must be employed to bring the alkalinity to a pH of above 7 to 9 (preferably about 9). Representative lower aliphatic 20 monocarboxylic acids and salts which can be advantageously employed are formic acid, acetic acid, propionic acid, butyric acid, the corresponding ammonium salts as well as carbonic acid and its corresponding ammonium salt.

25 The amount of metal salt which is employed in the treating solution can vary from 0.05 ounce per gallon to 10 ounces per gallon.

The metallization treatment in accordance with this invention is applicable to fibrous materials having thereon 30 an azoic dyeing in which the dye molecule contains an aromatic configuration which lends itself to the production of an o,o'-dihydroxy type of metallization. Such azoic dyeings may be produced in situ on the fiber in any conventional manner; e.g., by impregnating the fiber with 35 an azoic coupling component and then dyeing with a solution which contains an active diazo either in the form of a freshly prepared diazo or as a Fast Color salt solution. The dyeing may also be produced by printing the fiber with a paste which comprises a mixture of the diazo 40 amino compound and coupling component and exposing the printed fiber to conditions suitable for coupling.

45 The diazos and the coupling components employed are those which are free from solubilizing groups such as sulfonic and carboxylic acids and which produce dyes having hydroxy groups ortho to the azo linkage or groups which are convertible into hydroxy groups such as lower alkoxy, i.e., methoxy, ethoxy, propoxy and butoxy.

50 The diazos employed in this invention are those produced from any aromatic diazotizable amine which does not contain solubilizing groups such as sulfonic and carboxylic acids and includes all of the conventional aromatic and heterocyclic amines that are customarily employed in the preparation of azoic dyes. Unless the 55 coupler to be used contains the o,o'-dihydroxy configuration the amine should also have an o-hydroxy or lower alkoxy group ortho to the amine group. As examples of such diazotizable amines, the following are illustrative:

- o-anisidine;
- 60 5-chloro-o-anisidine;
- 5-nitro-o-anisidine;
- o-dianisidine;
- 4-benzamido-2,5-dimethoxyaniline;
- 2,5-dimethoxy-4-(p-nitrobenzeneazo)aniline;
- 65 4-cyano-2,5-dimethoxyaniline;
- 5-diethylsulfamyl-o-anisidine;
- 4-phenylamino-o-anisidine;
- 5-n-butylsulfamyl-o-hydroxyaniline;
- 5-amino-6-hydroxyquinoline;
- 70 2-hydroxy-4-nitroaniline;
- 2-hydroxy-5-nitroaniline;
- chlorotoluidines;

chloroaniline;  
dichloroaniline;  
trifluoromethylchloroaniline;  
4-nitro-o-anisidine;  
4-chloro-o-anisidine;  
5-chloro-4-nitro-o-anisidine;  
credisine;  
5-(butylsulfamyl)-o-anisidine;  
4-benzamido-2,5-diethoxyaniline;  
4-benzamido-5-methyl-o-anisidine.

5

10

In the case where the coupling component contains the o,o'-dihydroxy configuration, the above may be used, as also those free from the o-hydroxy and alkoxy configuration, e.g., p-chloroaniline, p-anisidine and benzidine.

The coupling components may, in general, be selected from the Naphthol AS compounds which are arylides of 2-hydroxy-3-naphthoic acid and related  $\beta$ -hydroxy carboxylic acid derivatives, acetoacetylides and related  $\beta$ -oxocarboxylic acid arylides and pyrazolones. However, other compounds may be employed which are capable of coupling to yield a component having the required metallizable group in ortho position to the azo linkage. Thus, in addition to the coupling components specifically set forth in the examples, the following coupling components may be employed:

15

20

2-naphthol,  
3-hydroxy-2-(2',5'-dimethoxy)naphthanilide,  
3-hydroxy-2-(N-naphthyl)naphthamide,  
3-hydroxy-2-(4'-chloro)naphthanilide,  
3-hydroxy-2-(N-2-methoxy-3-dibenzofuryl)naphthamide,  
3-hydroxy-anthraquinone-2-carbox-o-toluidide,

30

2-hydroxy-3-dibenzofurancarboxylic acid arylides such as 2-hydroxy-3-dibenzofuran(2',5'-dimethoxy)carboxanilide, bis(acetoacet)benzidine, bis(acetoacet)-tolide, acylacetanilides such as acetoacet-4-chloro-2,5-dimethoxy-anilide, 3-hydroxy-2-carbazole-carboxylic acid arylides such as 3-hydroxy-2-carbazole-(p-chloro)carboxyanilide, terephthaloyl bisacetoacet-(3'-chloro-2',4'-dimethoxy)-anilide, pyrazolones, such as 1-phenyl-3-methyl-5-pyrazolone, 3-hydroxy-2-naphthoic acid arylides, o-hydroxy-aniline  $\rightarrow$  resorcinol, 2-hydroxy-5-nitro-aniline  $\rightarrow$  resorcinol. In the case of the couplers in the last two examples listed, wherein the o-hydroxyazo linkage is present in the coupler per se, any ordinary diazo compounds may be employed, such as m-chloroaniline, o-nitroaniline, 1-amino-anthraquinone and 2-amino-4,4'-dichlorodiphenyloxide. Other azo couplers, such as the metallized compounds disclosed in United States Patent 2,135,433 and the unmetallized products thereof, and the like can also be employed.

35

The diazo may be supplied by an amine freshly diazotized by treatment with nitrite in the customary manner, or the diazo may be stabilized diazo, i.e., in the form of diazonium chloride or sulfate, or in the form of the diazo stabilized as a double salt, i.e., as a zinc chloride, boron trifluoride, tin chloride, naphthalenedisulfonic acid, etc.

45

As illustrative examples of Fast Color Salts, the following are illustrative:

40

50

55

60

65

70

75

#### Fast Blue Salt BN



#### Fast Blue Salt 2BN



#### Fast Red Salt BN



#### Fast Red Salt TRN



#### Fast Black Salt K



#### Fast Bordeaux Salt BD



#### Variamine Blue Salt BD



#### Fast Red Salt RL



#### Fast Red Salt FR



In practice, the fibrous material is first dyed or printed in conventional manner. Thus, the fiber may be padded with a solution of approximately 0.1 to 10 percent of coupler. The material dried and then treated with the diazo solution or the material may be impregnated in conventional manner with naphthol, hydroextracted or salt rinsed to remove excess naphthol and excess alkali, developed with a diazo solution and finished in customary manner. Alternatively, the textile material may be printed with a Rapidogen and then developed in acid or neutral steam.

After the dyeing or printing is completed, the dyed or printed material is metallized in accordance with the method of the invention for a period of time of from about 5 seconds to 10 minutes depending on the degree of metallization desired, at a temperature in the range of from 100 to 212° F. The metallizing solution contains per 1 part of metal salt, 1-4 parts of carbonic acid or a lower aliphatic carboxylic acid and 2-15 parts of ammonium hydroxide to provide an alkalinity to the solution of a pH of from above 7-9, and preferably closer to pH 9. The same result may be accomplished by the employment of the ammonium salts of the corresponding acids and any additional ammonium hydroxide necessary to control and maintain the pH of the solution in the range aforementioned.

The following examples will serve to illustrate some of the preferred embodiments of the invention; it being clearly understood, however, that these examples are merely illustrative and are not to be considered as a limitation of the invention.

## Example 1

A metallizing solution was made up as follows:

| Copper solution:            | Parts |
|-----------------------------|-------|
| Copper sulfate              | 70    |
| Water                       | 280   |
| Ammonium hydroxide, 26° Bé. | 430   |
| Glacial acetic acid         | 220   |

A cotton print produced in the usual manner from tetrazotized dianisidine and Naphthol AS was treated in 2 ounces of the above solution plus 1/2 ounce of ammonium hydroxide per gallon of added water at 150° F. for 10 seconds, rinsed and dried.

In comparison, a similar cotton print was treated in a solution which contained 0.5 ounce copper sulfate and 0.5 ounce acetic acid in 1 gallon water at 200° F. for 10 seconds, rinsed and dried. This method constitutes normal metallizing procedure as it is now practiced.

Metallization in case of the ammonia-containing metallizing bath was more efficient than in the case of the other bath as shown by better light fastness.

## Examples 2-10

A cotton print produced from tetrazotized dianisidine and Naphthol AS was treated at 200° F. for 1 minute in the following baths:

|                           | Example |     |     |     |     |     |     |     |     |  |
|---------------------------|---------|-----|-----|-----|-----|-----|-----|-----|-----|--|
|                           | 2       | 3   | 4   | 5   | 6   | 7   | 8   | 9   | 10  |  |
| Water (gallon)            | 1.0     | 1.0 | 1.0 | 1.0 | 1.0 | 1.0 | 1.0 | 1.0 | 1.0 |  |
| Copper sulfate (oz.)      | 0.5     | 0.5 | 0.5 | 0.5 | 0.5 | 0.5 | 0.5 | 0.5 | 0.5 |  |
| Ammonium acetate          | 3.0     | 5.0 | 3.0 |     |     |     |     |     |     |  |
| Ammonium hydroxide 26° Bé |         |     | 1.0 |     | 2.0 | 2.2 | 0.5 | 0.5 | 0.5 |  |
| Ammonium carbonate        |         |     |     | 2.2 |     |     |     |     |     |  |
| Acetic acid               |         |     |     |     | 1.5 | 2.8 |     |     |     |  |
| Ammonium formate          |         |     |     |     |     |     | 3.5 |     |     |  |
| Ammonium propionate       |         |     |     |     |     |     |     | 3.5 |     |  |
| Ammonium butyrate         |         |     |     |     |     |     |     |     | 3.5 |  |

In the above set of examples, cotton dyed with tetrazotized dianisidine coupled with Naphthol AS is treated in the solution at 200° F. for 1 minute, rinsed and dried. In all cases, metallization was satisfactory as shown by light fastness tests.

## Examples 11-14

|                           | Example |     |     |     |
|---------------------------|---------|-----|-----|-----|
|                           | 11      | 12  | 13  | 14  |
| Water (gallon)            | 1.0     | 1.0 | 1.0 | 1.0 |
| Copper sulfate (oz.)      | 0.5     | 0.5 | 0.5 | 0.5 |
| Ammonium hydroxide 26° Bé | 2.0     | 0.6 | 0.5 | 0.5 |
| Ammonium sulfate          |         |     | 3.0 |     |
| Ammonium chloride         |         |     |     | 2.5 |

In the above set of examples, cotton dyed with tetrazotized dianisidine coupled with Naphthol AS is treated in the solution at 200° F. for 1 minute, rinsed and dried. In no case was a good metallization obtained as the solution tended to become unstable and precipitate. The metallizations were dull, several tended to be bronzy and the dyeings lacked the high degree of light fastness imparted by the teachings of this invention.

This set of examples demonstrates that ammonium hydroxide alone or in combination with the stronger inorganic acid salts, is not satisfactory.

## Example 15

A print is made on cotton in the usual manner from 4-benzamido-5-methyl-o-anisidine diazotized and stabilized with sarcosine and Naphthol AS. This print is treated for 10 seconds at 200° F. in the copper solution of Example 1. Metallization was efficient as determined by the color and light fastness of the print.

## Example 16

10 A metallization was made as in Example 15, employing a print made in the usual manner from tetrazotized and stabilized dianisidine and Naphthol AS. The metallization was efficient as determined by shade and light fastness tests.

## Example 17

15 A metallization was made as in Example 15, employing a print made in the usual manner from diazotized and stabilized 5-methyl-o-anisidine and coupled with 3'-nitro-3-hydroxy-2-naphthalenilide. The metallization was 20 efficient as determined by shade and light fastness tests.

## Example 18

A metallization was made as in Example 15, employing a print made in the usual manner from 4-benzamido-5-methyl-o-anisidine diazotized and stabilized with methylytaurine and coupled with 4-(5-chloro-2-hydroxyphenyl-

azo) resorcinol. The metallization was efficient as determined by shade and light fastness tests.

## Example 19

Cotton was padded in the usual manner with a solution which consisted of 1.0 parts of the coupler of the formula:



55 2.0 parts glycol monoethyl ether, 1.6 parts caustic flake and 133 parts water. The material was dried and padded with a solution consisting of 4.0 parts 4-nitro-o-anisidine diazotized and stabilized with 1,5-naphthalene-disulfonic acid, 1.0 part Diazopon SS 833 (commercial dispersing agent), 1.0 part 50 percent acetic acid solution and 2.5 parts sodium acetate in 133 parts of water. After rinsing and drying, the material was metallized at 200° F. in the copper bath of Example 1 for 1 minute, rinsed and dried. The metallized reddish brown dyeing was much faster to light and washing than a similar dyeing metallized with copper sulfate and acetic acid alone.

## Example 20

Cotton material was padded as in Example 19 with a solution of coupler differing only in that 1.0 part of 70 the coupler of the formula:



was substituted for the coupler of Example 19. In padding with diazo, the solution consisted for 4.5 parts 2,5-dichloroaniline diazotized and stabilized with zinc chloride, 1 part Diazopon SS 833, 1 part acetic acid 50 percent solution and 1.5 parts sodium acetate in 133 parts of water. After rinsing and drying, the material was metallized at 200° F. in the copper bath of Example 1 for 1 minute, rinsed and dried. The metallized reddish brown dyeing was much faster to light and washing than a similar dyeing metallized in the usual manner in a copper sulfate-acetic acid solution.

*Example 21*

Cotton material was padded as in Example 19 with a solution of coupler differing only in that 1.0 part of the coupler of the formula:



was substituted for the coupler of Example 19. In padding with diazo, the solution consisted of 2.0 parts dianisidine tetrazotized and stabilized with zinc chloride, 1.0 part Diazopon SS 833, 0.5 part acetic acid 50 percent solution and 2.0 parts sodium acetate in 133 parts of water. After rinsing and drying, the material was metallized at 200° F. in the copper bath of Example 1 for 1 minute, rinsed and dried. The metallized reddish blue dyeing was much faster to light and washing than a similar dyeing metallized in the usual manner in a copper sulfate-acetic acid solution.

*Example 22*

A cobalt solution was made up as follows:

|                             | Parts |
|-----------------------------|-------|
| Cobalt chloride             | 70    |
| Water                       | 280   |
| Ammonium hydroxide, 26° Bé. | 430   |
| Glacial acetic acid         | 220   |

As in Example 1, a cotton print produced from tetrazotized dianisidine and Naphthol AS was treated in 2 parts of the above solution and 1/2 part of ammonia in 133 parts of water at 150° F. for 10 seconds, rinsed and dried.

Metallization was efficient and the dyeing had a better shade and improved light fastness over a similar metallization made using 0.5 part of cobalt chloride and 0.5 part acetic acid in 133 parts of water at 200° F. for 10 seconds.

*Example 23*

A nickel solution was made up as follows:

|                            | Parts |
|----------------------------|-------|
| Nickel chloride            | 70    |
| Water                      | 280   |
| Ammonium hydroxide 26° Bé. | 430   |
| Glacial acetic acid        | 220   |

As in Example 1, a cotton print produced from tetrazotized dianisidine and Naphthol AS was treated in 2 parts of the above solution plus 1/2 part ammonia in 133 parts of water at 150° F. for 10 seconds, rinsed and dried.

Metallization was efficient and the dyeing had a better shade and improved light fastness over a similar metallization made using a solution of only 0.5 part nickel chloride, and 0.5 part acetic acid in 133 parts water at 200° F. for 10 seconds.

Various modifications of the invention will occur to persons skilled in the art. Thus, it is evident in lieu of the compounds of the specific examples, any of the com-

pounds mentioned above can be employed with similar results. Therefore, it is not intended that the invention be limited in the patent granted except as necessitated by the appended claims.

5. What is claimed is:

1. In the method of after-treating fibrous materials dyed with an azoic dye free of solubilizing groups and containing in o,o'-positions relative to an azo linkage groups capable of conversion to a complex metal compound, the improvement which comprises treating said dyed fibrous material with an alkali-ion-free aqueous alkaline solution having a pH in the range of above 7-9, containing (1) a metallizing compound of the group consisting of salts and hydroxides of copper, cobalt and nickel capable of forming a metal complex with said azoic dye, (2) an ammonium salt of the formula:



20 wherein X represents a member selected from the group consisting of hydroxyl, hydrogen and alkyls having 1 to 4 carbon atoms and, (3) such amount of ammonium hydroxide as is necessary to maintain the pH of the solution in said range.

2. In the method of after-treating fibrous materials dyed with an azoic dye free of solubilizing groups and containing in o,o'-positions relative to an azo linkage groups capable of conversion to a complex metal compound, the improvement which comprises treating said dyed fibrous material with an alkali-ion-free aqueous alkaline solution having a pH in the range of above 7-9, containing (1) a metallizing compound of the group consisting of salts and hydroxides of copper, cobalt and nickel capable of forming a metal complex with said azoic dye and, (2) ammonium salts of acids selected from the group consisting of carbonic acid and lower aliphatic monocarboxylic acids.

3. In the method of after-treating fibrous materials dyed with an azoic dye free of solubilizing groups and containing in o,o'-positions relative to an azo linkage groups capable of conversion to a complex metal compound, the improvement which comprises treating said dyed fibrous material with an alkali-ion-free aqueous alkaline solution having a pH in the range of above 7-9, containing (1) a metallizing compound of the group consisting of salts and hydroxides of copper, cobalt and nickel capable of forming a metal complex with said azoic dye, (2) ammonium salts of acids selected from the group consisting of carbonic acid and lower aliphatic monocarboxylic acids and, (3) ammonium hydroxide in an amount sufficient to provide the aforesaid alkalinity.

4. The method according to claim 2 wherein the metallizing compound is copper sulfate and the ammonium salt is ammonium acetate.

5. The method according to claim 2 wherein the metallizing compound is copper sulfate and the ammonium salt is ammonium carbonate.

6. The method according to claim 2 wherein the metallizing compound is copper sulfate and the ammonium salt is ammonium formate.

7. The method according to claim 2 wherein the metallizing compound is copper sulfate and the ammonium salt is ammonium propionate.

8. The method according to claim 2 wherein the metallizing compound is copper sulfate and the ammonium salt is ammonium butyrate.

9. The method according to claim 3 wherein the metallizing compound is copper sulfate and the acid is glacial acetic acid.

10. The method according to claim 3 wherein the metallizing compound is cobalt chloride and the acid is glacial acetic acid.

11. The method according to claim 3 wherein the

metallizing compound is nickel chloride and the acid is  
glacial acetic acid.

12. The method of claim 1 in which the dyed fibrous  
material is treated with the solution at a temperature of  
about 100-212° F. for about 5 seconds to ten minutes. 5

13. The method of claim 2 in which the dyed fibrous  
material is treated with the solution at a temperature of  
about 100-212° F. for about 5 seconds to ten minutes.

14. The method of claim 3 in which the dyed fibrous  
material is treated with the solution at a temperature of 10  
about 100-212° F. for about 5 seconds to ten minutes.

## References Cited by the Examiner

## UNITED STATES PATENTS

|           |         |                        |        |
|-----------|---------|------------------------|--------|
| 1,853,418 | 4/1932  | Hentrich et al. -----  | 8-42   |
| 2,148,659 | 2/1939  | Straub et al. -----    | 8-42   |
| 2,673,200 | 3/1954  | Ruchstuhl et al. ----- | 8-74 X |
| 2,768,055 | 10/1956 | Streck -----           | 8-42   |

NORMAN G. TORCHIN, Primary Examiner.

D. LEVY, Assistant Examiner.